

Oct. 11, 1932.

L. L. JONES

1,881,644

ELECTRON DISCHARGE CATHODE

Filed Feb. 28, 1929

Fig. 1.



Fig. 2.



INVENTOR  
Lester L. Jones

BY

*Caravaghi & Jones*  
ATTORNEYS

## UNITED STATES PATENT OFFICE

LESTER L. JONES, OF ORADELL, NEW JERSEY

## ELECTRON DISCHARGE CATHODE

Application filed February 28, 1929. Serial No. 343,255.

This invention relates to electron discharge devices or tubes and has special reference to the provision of a novel cathode structure for electron discharge devices or tubes.

The problem of constructing cathode elements embodying heaters for the oxide emitters in electron discharge tubes has been fraught with many difficulties and has led to severe limitations in the design of electron discharge devices or vacuum tubes. It is desirable, for example, to coat the thermionically active material or oxide emitter on a metal such as nickel, molybdenum or tungsten. The resistances of these metals are too low, however, to generate the required amount of heat in the current and voltage ranges desirable unless the metal be drawn into extremely fine wire, or unless long lengths be used. The drawing of these metals into filaments gives rise to the necessity for providing filament supporting structures to prevent the sagging and vibrational motions of the fine filaments and such filament supporting structures undesirably occupy considerable space in the vacuum tube.

Where the cathodes are of the so-called uni-potential heated type, it has been necessary to provide a considerable mass of insulating material between the heater and the electron emitting cathode surface, the heater comprising in such uni-potential cathode structures an element electrically distinct from the electron emitting cathode surface. This type of uni-potential cathode gives rise to heater burnouts and is especially troublesome in the construction of relay tubes for broadcast receivers due to the relatively long time required to heat up the cathode to the emitting temperature.

In the construction of electron discharge tubes in which the heaters are energized by alternating current, another problem resides in the importance of confining the electrostatic field due to the voltages in the heater into a region outside the path of the electron flow. It is also important to minimize the magnetic field due to the heater currents especially in the region of the electron current flow.

The prime desideratum of my present in-

vention centers about the provision of a new cathode structure in which the above disadvantages incident either to the filamentary or indirectly heated prior art types of cathode structures are effectively obviated and which is characterized by new advantages and by the opening up of a new field of design in the electron discharge tube and allied arts. Among these new advantages which comprise objects of the present invention are the construction of a cathode element including a heater which defines a rigid self-supporting structure devoid of any insulating material, the further provision of a heater which is extremely compact and preferably of a long cylindrical form, the further provision of a heater in which all of the parts are mechanically integral, are in intimate contact with one another and therefore free from any loose parts, the still further provision of a cathode heater in which the heat distribution is uniform to the surface of application, and the construction of a heater in which the magnetic and capacitive fields due to the heater current and voltage are at a minimum. These advantages and the accomplishments of these objects lead to important results in many fields; and in the present application I will relate the especial advantages which appertain to the production of cathodes for use in electron discharge devices or vacuum tubes.

To the accomplishment of the foregoing and such other objects as will hereinafter appear, my invention consists in the elements and their relation one to the other, as herein-after more particularly described and sought to be defined in the claims; reference being had to the accompanying drawing which shows the preferred embodiments of my invention, and in which:

Fig. 1 is a circuit diagrammatic view of an electron discharge device embodying my invention and showing one manner of its use;

Fig. 2 is a generalized structural view of an electron discharge tube showing my invention applied thereto; and

Fig. 3 is a view taken on an enlarged scale and showing in detail the cathode structure of the present invention.

Having reference now more in detail to

the drawing and referring first to Fig. 3 thereof, the cathode structure of the invention comprises a unitary element embodying spaced conducting electrodes 10 and 11, one of which provides the electron emitting surface and a resistor element 12 defining the heater disposed between and conductively integral with the electrodes 10 and 11. In the preferred embodiment of the invention, the 5 electrode 10 comprises a fairly rigid central core made, for example, of copper, nickel, tungsten, etc., having a diameter approximately 1/100 of its length, the resistor element 12 comprises a coating of a high resistance material coated over and covering the core 10, and the electrode 11 comprises a conductive film of such a metal as silver, copper or nickel which preferably is electroplated over the resistance coating 12 and 10 forms a cylindrical shell which receives the outer coating 13 of a thermionically active 15 preparation or oxide emitter.

In the design and construction of this cathode element it is contemplated that the 20 conductivity of the core 10 and of the electroplated shell 11 be very high as compared to the conductivity of the resistance layer or coating 12 therebetween. Heat is therefore generated in the resistance layer and substantially 25 the entire voltage drop occurs in the resistance layer. Due to this construction, the electrostatic field incident to the heater voltage is therefore confined to within the heater element and therefore to a region outside 30 the path of the electron flow. If the current be led in and from the electrodes 10 and 11 by means of the conductors 14 and 15 attached to the electrodes, as shown in Fig. 3 35 of the drawing, substantially no magnetic field is created because the return current is led back to the point of origin along the path in extremely close spacial relationship to the outgoing path. Thus the magnetic field due 40 to the heater currents is minimized especially in the region of the electron current flow. It 45 will also be noted that that part of the current which is used for heating near the heater terminals does not travel through the more remote portions of the heater, and therefore the remote portions have lesser currents and the residual magnetic field in their vicinity 50 therefore becomes negligible. This is in marked contrast to prior art types of heaters in which the heater current flows through the 55 whole length of the heater and in which, therefore, residual magnetic fields are at a maximum.

The cathode unit or heater as thus constructed provides, moreover, a self-supporting structure, all the elements of which are conductively integral eliminating, therefore, the need or use for supporting members or insulating material which characterize cathode units or heaters of the prior art. The 60 construction of a self-supporting heater in

this fashion gives rise to a minimum of material to be heated and therefore to extremely fast heating of the cathode and permits the construction of a cathode unit which may be used in an electron discharge tube with the 65 elimination of the considerable loss of space incident to structures of the prior art. Because of the extremely quick heating of the cathode, the time for starting the tube is reduced to the order required for the filamentary types of cathode of the prior art. The compacting of the cathode confining the same into a minimum of space, permits of the use 70 of much smaller grids and plates with consequent advantages in the reduction of inter-electrode capacities of the electron discharge 75 device. All of the parts of the heater being conductively integral are in intimate contact, and therefore the unit as a whole is 80 free from any loose parts. It will be apparent, moreover, that the heat distribution is 85 uniform to the surface of application.

In the preferred construction, the resistor element 12 comprises a high resistance material of the kind described and claimed in 90 the application of Lester L. Jones, et al., Serial No. 167,583, filed February 11, 1927, and the electroplated outer shell 11 is applied to the resistor coating 12 preferably in 95 the manner described and claimed in the application of Lester L. Jones and Joseph A. Flanzer, Serial No. 260,987, filed March 12, 1928. As set forth in said application, the resistance coating 12 is composed of a finely divided graphite mixed with a binder and vehicle consisting of a metallic phosphate. In compounding the resistance material, the graphite, preferably a colloidal graphite, is mixed with a solution of aluminum in phosphoric acid to form a freely flowing 100 paint. The aluminum in the phosphoric acid produces an aluminum phosphate; and in the preparation of the aluminum phosphate it has been found desirable to add 105 aluminum to the phosphoric acid in such an amount as just fails to produce a precipitate. Addition of more than this amount, which would produce a precipitate, is undesirable 110 because of the presence in the paint of large particles formed by the precipitate which interfere with the production of a smooth uniform film. On the other hand, the addition of an insufficient quantity of aluminum or aluminum phosphate is undesirable mainly 115 because of the more highly acid condition of the resulting paint, which tends to destroy the colloidal nature of the graphite, causing clotting of the paint with streakiness in the film. It is therefore preferred to use a solution of aluminum in phosphoric acid in a slight excess of phosphoric acid, aluminum being added in such an amount as just fails to produce a precipitate. The aluminum phosphate may also be prepared by the 120 addition of C. P. aluminum phosphate to 125

phosphoric acid in sufficient quantity to just avoid the formation of any precipitate.

The paint thus compounded is then applied to the conductive core 10 by means of a brush or by dipping or by any other method. After being applied the embryo unit thus formed is subjected to a heat treatment which produces a tough and durable coating or film having a relatively high resistance. This coating (12) is then electroplated to the required thickness, usually of the order of several thousandths of an inch of conducting metal which may be silver, copper or nickel. The paint coating 12 is found to adhere very firmly to the conductive core 10 and forms a firm basis or support for the deposited or plated metal film. In affixing the terminals 14 and 15 to the electrodes of the cathode unit, it is preferred to reinforce one end of the electrode shell 11 with a ring 16 of additional thickness and this may be accomplished by the method of spot electroplating the shell 11, as described and claimed in the copending application of Joseph A. Flanzer, Serial No. 223,264, filed October 1, 1927. The lead wires or conductors 14 and 15 may then be spot welded, one to the end of the core 10 and the other to the reinforced spot plated ring 16. In some cases the reinforcement may be placed at the middle of the heater instead of at one end thereof.

In Fig. 2 of the drawing, I show diagrammatically the structural inter-relation between the cathode unit of my invention and the other elements of an electron discharge device illustrating some of the advantages hereinbefore outlined when the heater is used in an electron discharge tube. This electron discharge device comprises the usual evacuated vessel 17 provided with the cathode C of the present invention, the said cathode being surrounded by the grid structure G which is interposed between the cathode and the plate P.

In Fig. 1 of the drawing, I show diagrammatically a vacuum tube embodying the cathode of the present invention depicting the manner of connecting such a vacuum tube in a relay circuit. As shown, the electrodes 10 and 11 of the cathode unit are connected to a battery A, the electrode 11 and the grid G comprising the electrodes of an input circuit I which is fed from a transformer T, said input circuit being provided, for example, with a battery C. The electrode 11 and the plate P form the electrodes of an output circuit O which in turn is connected to a transformer T', and which output circuit is supplied with a battery B. The use and operation of such amplifier or relay circuits, as shown in Fig. 1 of the drawing, is well known to the art and need not be further detailed.

The manner of making cathodes or heaters

of the present invention and the making of electron discharge devices embodying such cathodes or heaters, and the many advantages in the manufacture and use thereof will in the main be fully apparent from the above detailed description thereof. It will be further apparent that while I have shown and described my invention in the preferred forms, many changes and modifications may be made in the structure disclosed without departing from the spirit of the invention, defined in the following claims.

I claim:

1. A heater comprising a conductive core, a conductive shell having one closed end and surrounding said core, a resistor element disposed between and forming the sole conductive path between said core and shell, and lead-in wires connected to the core and the shell at one end only of the said heater. 80

2. A unitary heater structure comprising a rigid highly conductive metallic core and support, a thin film or coating of high resistance material over said core, a highly conductive film of metal over said resistance coating, the resistance film forming the sole conductive path between the support and the metallic film, an electron emitter coating over said film, and lead-in wires connected to the metallic core and the metallic film at 95 one end only of said heater.

3. An electron emitting cathode comprising a conductive core defining one cathode electrode, a resistor coating thereon forming the cathode heater, and a conductive shell having one closed end surrounding said resistor coating and defining the other cathode electrode, said resistor forming the sole conductive path between the core and the shell. 106

4. A unit-potential cathode for low powered electron emission tubes comprising a central highly conductive wire or rod, a thin heater resistance surrounding the rod, a thin highly conductive metallic shell surrounding the heater resistance, the resistance material forming the sole conductive path between the rod and the shell, and lead-in wires connected to the rod and the shell at one end only of said rod and shell whereby a self-supporting rigid cathode is provided having a small diameter and small mass for low heat radiation loss and quick heating. 110

5. A cathode for low powered electron emission tubes comprising a highly conductive wire or rod, a high resistance film coated on the rod, a highly conductive metallic shell plated over the resulting resistance coating, the resistance material forming the sole conductive path between the rod and the shell, a thermionically active material applied to the said metallic shell, and lead-in wires connected to the rod and the shell at one end only of said rod and shell. 125

6. A uni-potential cathode for low powered electron emission tubes comprising a 130

central highly conductive wire or rod, a carbonaceous high resistance film coated on the rod, a highly conductive metallic shell plated over the resulting resistance film, the resistance material forming the sole conductive path between the rod and the shell, a thermionically active material applied to the said metallic shell, and lead-in wires connected to the rod and the shell at one end only of said rod and shell, whereby a self-supporting rigid cathode is provided having a small diameter and small mass for low heat radiation loss and quick heating.

7. A cathode comprising a highly conductive wire or rod, a heater resistance surrounding the walls and one end of the rod, and a highly conductive metallic shell placed over the walls and end of the heater resistance, said resistance being in intimate contact with said conductors and forming an electrical path therebetween.

8. A cathode for low powered electron emission tubes comprising a highly conductive wire or rod, a high resistance film coated entirely around the walls and one end of the rod, a highly conductive metallic shell plated on the walls and end of the resulting resistance coating, and a thermionically active material applied to the said metallic shell.

9. A cathode for low powered electron emission tubes comprising a highly conductive wire or rod, a carbonaceous high resistance film coated entirely around the walls and one end of the rod, and a highly conductive metallic shell plated on the walls and end of the resulting resistance coating.

10. A non-magnetic uni-potential cathode for low powered electron emission tubes comprising a central highly conductive wire or rod, a carbonaceous high resistance film coated entirely around the walls and one end of the rod, a highly conductive metallic shell plated on the walls and end of the resulting resistance coating, and a thermionically active material applied to the said metallic shell, whereby a self-supporting rigid cathode is provided having a small diameter and small mass for low heat radiation loss and quick heating.

50 Signed at New York in the county of New York and State of New York this 26th day of February A. D. 1929.

LESTER L. JONES.